

C. M. STEIN.

ANNEALING,

APPLICATION FILED AUG. 18, 1919.

1,388,976.

Patented Aug. 30, 1921.

Fig. 2



Fig. 1



Inventor

Charles M. Stein  
by *Charles M. Stein*  
*Sam J. Stelle* atty.

# UNITED STATES PATENT OFFICE.

CHARLES M. STEIN, OF PARIS, FRANCE, ASSIGNOR TO SOCIETE ANONYME DES APPAREILS DE MANUTENTION ET FOURS STEIN, OF PARIS, FRANCE, A CORPORATION OF FRANCE.

## ANNEALING.

1,388,976.

Specification of Letters Patent. Patented Aug. 30, 1921.

Application filed August 18, 1919. Serial No. 318,169.

To all whom it may concern:

Be it known that I, CHARLES M. STEIN, citizen of the French Republic, residing at Paris, Department of the Seine, in France, and whose post-office address is 31 Boulevard Péreire, in the said city, have invented certain new and useful Improvements in or in Connection with Annealing; and I do hereby declare the following to be a full, clear, and exact description of the invention, such as will enable others skilled in the art to which it appertains to make and use the same.

In the process of annealing it is usual to effect the operations in an oxidizing atmosphere and to protect the articles from the deleterious action of this atmosphere by placing them in closed boxes or receptacles.

This method has serious disadvantages as, in the first place, it necessitates the consumption of fuel additional to that required to heat the articles, to heat the boxes or receptacles and, in the second place, the boxes or receptacles wear out rapidly and require frequent renewal.

The present invention has for its object to enable the process of annealing to be carried out in an improved manner in a non-oxidizing atmosphere and without the employment of boxes or receptacles.

Furnaces have been proposed in which the process of annealing is carried out in a non-oxidizing atmosphere and without the employment of boxes or receptacles, but the present invention is differentiated therefrom in that the process is carried out in a muffle and in a non-oxidizing atmosphere consisting of the gas employed to heat the muffle which is introduced under pressure within the muffle and subsequently consumed externally thereto.

Referring now to the accompanying drawings:

Figure 1 is a longitudinal section; Fig. 2 is a cross section of the annealing furnace.

The directions of flow of the air, gas and products of combustion are indicated by the single, double and triple-headed arrows respectively.

The articles 1 to be annealed, for example, thin iron plates, are placed on small trucks 2 and are run on rails or rollers 3 into the muffle 4.

The furnace is heated by gas supplied

from an independent gas producer. This gas, which consists principally of carbon monoxide and nitrogen, provides the neutral or non-oxidizing atmosphere and is led into the muffle 4 under pressure through a duct 5, passes through the muffle, driving out, at the commencement of the operation, the inclosed air; the gas passes from the muffle 4 through openings 6 in the side walls, after which it encounters air heated by passage through regenerators 7. Combustion of the gas thus takes place without the muffle 4, which is heated over the whole of its external surface. The products of combustion pass through vertical ducts into horizontal ducts 8 at the upper part of the furnace structure and flow from thence to the regenerators 7, which are heated thereby.

When the heating has continued for a sufficient time to insure the annealing of the articles, the trucks 2 are run out of the muffle 4 and other articles introduced.

The invention is not limited to the details of construction of furnace illustrated.

I claim:

1. An annealing furnace comprising a muffle adapted to receive the articles to be annealed, a combustion chamber immediately surrounding said muffle, means for admitting a non-oxidizing gas directly into said muffle, openings in the wall of said muffle for allowing said gas to pass through the muffle into the surrounding chamber and means for admitting air into said surrounding chamber to mix with said non-oxidizing gas forming a combustible mixture to be burnt in said chamber for heating said muffle.

2. An annealing process whereby the articles to be annealed are placed within a muffle and annealed in a non-oxidizing atmosphere consisting of the gas employed to heat the muffle, which gas is introduced directly therein under pressure and subsequently passes through openings in the wall of the muffle and is mixed with air and consumed in the combustion chamber immediately surrounding said muffle.

In testimony whereof I affix my signature in presence of two witnesses.

CHARLES M. STEIN.

Witnesses:

CHAS. P. PRESSLY,  
EMILE KLOH.